

May 8, 1923.

1,454,066

H. A. MYERS

MOLD AND PROCESS FOR CASTING MATERIALS

Filed April 15, 1921



FIG. 3.

INVENTOR

*Hubert A. Myers  
by  
Owen, Owen & Hampton*

## UNITED STATES PATENT OFFICE.

HUBERT A. MYERS, OF TOLEDO, OHIO, ASSIGNOR TO THE HUBERT A. MYERS COMPANY, OF TOLEDO, OHIO, A CORPORATION OF OHIO.

## MOLD AND PROCESS FOR CASTING MATERIALS.

Application filed April 15, 1921. Serial No. 461,623.

To all whom it may concern:

Be it known that I, HUBERT A. MYERS, a citizen of the United States, and a resident of Toledo, in the county of Lucas and State 5 of Ohio, have made an invention appertaining to Molds and Processes for Casting Materials; and I do hereby declare the following to be a full, clear, and exact description of the invention, such as will enable others 10 skilled in the art to which it appertains to make and use the same, reference being had to the accompanying drawings, and to the characters of reference marked thereon, which form a part of this specification.

15 My invention has for its object to provide a mold wherein materials that are rendered plastic or fluid by heat, and which are structurally injured by an improper rate of cooling, may be rapidly cast and yet produce the 20 best possible structural condition within the castings. A great variety of materials may be cast in the molds involving my invention, such as ferrous metals, brass of relatively high fusibility, and silica compounds and 25 mixtures, such as glass. The invention is particularly valuable in casting ferrous metals when it is desired to rapidly produce soft metal castings having a substantially uniform structure throughout. The invention 30 particularly provides a process for casting metals having high fusibility wherein a high substantially uniform temperature of the mold is maintained by the use of a metal of low fusibility, and preferably one 35 having a high boiling point, a high vaporizing point, and a high heat conductivity.

Also my invention has for its object to provide a means for constantly feeding to the molding surface of the molds a material 40 that will protect the mold from the action of the heated metal of the castings.

To illustrate a practical application of the invention I have selected a mold containing my invention as an example of such molds 45 in which the process involving my invention may be conducted. The mold selected for purposes of illustration is shown in the accompanying drawing and together with the process will be described hereinafter.

50 Figure 1 of the drawing illustrates a perspective view of the mold. Fig. 2 illustrates a vertical sectional view of the mold, and Fig. 3 illustrates a transverse sectional view of the mold.

The mold is a metal mold and is formed 55 of two parts 1 that correspond to the drag and the cope of the ordinary foundry flask. They are formed with registering parts that contain the molding cavity 2 of the mold and the sprue hole 3 leading thereto. The 60 registering parts may be formed of two iron plates 4, one or both of which may be provided with suitable recesses or ridges according to the configuration of the article to be cast within the mold. The portions of the 65 plates 4 that form the cavity 2 are preferably of substantially uniform thickness so as to produce a uniform heat conductivity from the surface of the cavity through the plates. The cavity 2 is jacketed by chambers 5 located in the parts 1 of the mold. The chambers 5 are contained between the plates 4 and the side walls 6 of each of the parts 1 of the mold. The chambers 5 are thus separated from the cavity 2 by the 75 plates or walls 4. If desired, the plates 4 may be formed integral with the tops 7 of the parts 1.

The chambers are filled with a material 80 that will maintain the walls of the cavity 2 of the mold at a high temperature, and as far as possible maintain the temperature uniform and constant. Such a material should therefore be heat conductive and preferably heat convective. A heated liquid 85 material having boiling and vaporizing points above 300° F. may be used, which will remove by convection the excessive heat introduced into the mold with the molten material to be cast, and nevertheless will 90 keep the surface of the cavity at a high temperature. If the heat regulating medium has a comparatively low vaporizing point the chambers may be sealed to prevent the loss of the material. A metal of low fusibility 95 may be used, if it has comparatively high boiling and vaporizing points. I find it preferable to use lead as the medium for controlling the heat of the surfaces of the cavity, since lead not only has low fusibility and high boiling and vaporizing points but has a comparatively high conductivity, and while in the molten state it has high fluidity, or low viscosity. The lead will be melted by the heat of the material cast in the mold 100 and will carry away the heat of the casting while in the mold by conduction and convection at the proper rate, and yet maintain 105

the walls of the cavity at a high temperature for each pouring.

The material used for controlling the temperature of the walls of the cavity is poured, 5 while in a liquid state, into the chambers 5 through openings, such as those shown at 9. The openings may be closed by suitable covers or plugs 10 to prevent entrance of 10 the material to be cast into the chambers, and, if the material for controlling the temperature has a vaporizing point such that 15 the heat to which it is subjected vaporizes it, the vapor will be retained in the chambers by thus sealing them.

15 Any suitable means may be used for closing and opening the molds, such as the hinged bars 8 that are attached to the parts 1 of the mold.

The material to be cast is poured into 20 the cavity through the sprue hole 3, and the heat of the material will be conducted through the thin walls of the cavity to the lead, if lead is used, which will either maintain the lead in a molten condition, or will 25 melt the lead if it is solid. The parts of the mold may be separated and the casting discharged as soon as the latter has become sufficiently solid or strong to maintain its 30 form, or it may be permitted to remain in the mold until it has cooled throughout to the temperature of the mold. The temperature of the wall of the cavity throughout the area of the surfaces will be maintained between the melting and boiling points of 35 the lead, it being cooled only by the heat that may be conducted through the lead, which would be the major portion of the heat, and the heat that may be conducted along the plates 4 to the exterior of the 40 mold. The walls of the sprue hole 3 will also be maintained to near the temperature of the walls of the cavity 2, and consequently the material cast in the mold will come into immediate contact with a surface that 45 is nearly as high in temperature as that of the cavity.

The temperature of the walls of the cavity, and that of the heat conveying medium, may be controlled by the rate at which the 50 pourings are made and the castings ejected. Consequently, it is possible to maintain the cavity walls at a temperature slightly above the melting point of the lead, if lead is used, or the cavity walls may be maintained at 55 still higher temperatures by a corresponding increase in the rapidity of the pourings.

If it is desired to raise the walls of the cavity to a high temperature, the mold may be subjected to the heat produced by the gas 60 burners 11. This will keep the walls of the cavity and of the sprue hole, by reason of convection of the fluid, substantially at a uniform high temperature, and localization of the intense heat of the burners, so far as 65 the walls of the cavity are concerned, will

be avoided. If the intensity of the heat produced by the burners is sufficient to cause the lead to approach its boiling point, the temperature of the walls of the cavity will be maintained substantially constant notwithstanding the rate at which the pourings are made and the castings ejected.

Where ferrous metals are cast in the molds the uniform high temperature of the molding surfaces and the uniform rate of conductivity from the casting is very desirable to prevent local crystallization or formation of white metal or cementite in the castings. Similar molds may be used for casting other materials, provided, of course, they are manipulated according to the character of the material to be cast. To produce soft iron castings the temperature of the mold should be raised and maintained at a relatively high temperature, while for casting 85 glass it may be found desirable to heat the mold prior to the pouring, and then allow it to partially cool before discharging the article. The volume and the conductivity of the metal or other material in the chambers 90 of the mold will permit a uniform cooling of the glass until it is sufficiently cooled to be removed or ejected from the mold or allowed to be passed to a suitable tempering leer.

95 In casting certain materials the walls of the cavity and the sprue hole may be surfaced or impregnated with suitable materials to form protective films or coatings to prevent adherence of the material cast 100 in the mold to the material of which the walls of the cavity are formed, or to modify or protect the surfaces of the castings, such as to render them smooth. When ferrous metals are cast the molding surfaces may be 105 coated with black wash or graphite or lamp black. If it is desired, the walls of the cavity may be surfaced or impregnated with zinc. If the walls of the cavity are formed of iron, zinc or zinc alloy may be inserted 110 in the chambers 5 alone or together with the lead and the walls of the cavity will draw from the reservoirs of zinc formed by the chambers, by absorption and by the high 115 temperature produced at the molding surface of the cavity, and thus zinc and zinc oxide will be supplied to the surface, which will form a protective coat or gas film at each pouring, as well as a partial protective coating of zinc oxide that will be formed on the 120 surface of the cavity upon the removal of the casting. If the chambers 5 are closed, and the walls of the cavity are pregnable to zinc, the vapor pressure will coat with such absorptive power that the walls may have 125 for the zinc, to supply the zinc to the molding surface of the cavity and the sprue hole. This will effectively prevent adherence of the ferrous metals cast in an iron mold notwithstanding the rapidity of the castings. 130

It is preferable to use lead at all times because of the comparatively high boiling point that lead has.

I claim:

5. 1. In a mold for casting materials, the mold having a chamber and a molding cavity, a wall separating the chamber and the cavity, the chamber containing a material having a boiling point above 1,000° F. 70
10. 2. In a mold for casting materials, the mold having a chamber and a molding cavity, a wall separating the chamber and the cavity, the chamber containing a metal of low fusibility. 75
15. 3. In a mold for casting materials, the mold having a chamber and a molding cavity, a wall separating the chamber and the cavity, the chamber containing a metal of low fusibility and high vaporizing point. 80
20. 4. In a mold for casting materials, the mold having a chamber and a molding cavity, a wall separating the chamber and the cavity, the chamber containing a metal of low fusibility and high boiling and vaporizing points. 85
25. 5. In a mold for casting materials, the mold having a chamber and a molding cavity, a wall separating the chamber and the cavity, the chamber containing a metal of low fusibility, and means for heating the metal. 90
30. 6. In a mold for casting materials, the mold having a chamber and a molding cavity, a wall separating the chamber and the cavity, the chamber containing lead. 95
35. 7. In a mold for casting materials, the mold having a chamber located in proximity to the matrix of the mold and containing lead, means for heating the lead. 100
40. 8. In a mold for casting metals, the mold having a chamber and a molding cavity, a wall for separating the chamber from the cavity, the molding surface of the cavity surfaced with a metal gasifiable below the 105
45. temperature of the melting point of the metal cast, and the chamber containing a metal of low fusibility. 110
50. 9. In a mold for casting metals, the mold having a chamber and a molding cavity, a wall for separating the chamber from the cavity, the molding surface of the cavity surfaced with a metal gasifiable below the temperature of the melting point of the metal cast, the chamber containing lead. 115
55. 10. In a mold for casting metals, the mold having a chamber and a molding cavity, a wall for separating the chamber from the cavity, the molding surface of the cavity surfaced with a metal gasifiable below the temperature of the melting point of the metal cast, and the chamber containing a metal of low fusibility and the said gasifiable metal. 120
60. 11. In a mold for casting metals, the mold having a chamber and a molding cavity, a wall for separating the chamber from the cavity, the molding surface of the cavity impregnated with zinc and the metal of low fusibility containing zinc. 125
65. 12. In a mold for casting metals, the mold having a chamber and a molding cavity, a wall for separating the chamber and the cavity, the molding surface of the cavity surfaced with a metal gasifiable below the temperature of the melting point of the metal cast, the chamber containing lead and the gasifiable metal. 130
13. In a mold for casting metals, the mold having a chamber and a molding cavity, a wall for separating the chamber and the cavity, the molding wall of the cavity impregnated with zinc, and the chamber containing zinc. 135
14. In a mold for casting metals, the mold having a chamber and a molding cavity, a wall for separating the chamber and the cavity, the molding surface of the cavity impregnated with zinc, and the chamber containing lead and zinc. 140
15. In a mold for casting metals, the mold having a molding cavity and a closed chamber, a wall for separating the chamber and the cavity, the chamber containing a metal gasifiable below the melting point of the metal cast. 145
16. In a mold for casting metals, the mold having a molding cavity and a closed chamber, a wall for separating the chamber and the cavity, the wall impregnated with a metal gasifiable below the temperature of the metal cast, and the chamber containing the said gasifiable metal. 150
17. In a mold for casting metals, the mold having a molding cavity and a closed chamber, a wall for separating the chamber and the cavity, the wall impregnated with a metal gasifiable below the temperature of the metal cast, and the chamber containing the said gasifiable metal and a metal of low fusibility. 155
18. In a mold for casting materials, the mold having chambers substantially surrounding the matrix of the mold, the chambers containing metal having low fusibility, the walls of the cavity impregnated with a metal gasifiable below the temperature of the melting point of the material cast, and the metal of low fusibility containing the gasifiable metal. 160
19. In a mold for casting metals, the mold having chambers surrounding the matrix of the mold, the chambers containing metal having low fusibility, the walls of the cavity impregnated with zinc and the metal of low fusibility containing zinc. 165
20. In a mold for casting metals, the mold having chambers substantially surrounding the matrix of the mold, the chambers containing lead, the walls of the molding cavity impregnated with a metal gasifiable below the temperature of the melting point of the metal cast. 170

the metal cast, and the lead containing additional amounts of the gasifiable metal.

21. In a mold for casting materials, the mold having chambers substantially surrounding the matrix of the mold, the chambers containing lead and zinc, the walls of the cavity impregnated with zinc.

22. The process of casting fusible material in a mold which consists in maintaining the walls of the molding cavity at a high temperature by a heated metal of low fusibility located outside of the walls of the cavity, and introducing the material into the cavity.

23. The process of casting materials in a mold which consists in maintaining the walls of the molding cavity at a substantially uniform high temperature by a heated metal of low fusibility substantially surrounding the walls of the cavity, and introducing the material into the cavity.

24. The process of casting materials in a mold which consists in maintaining the walls of the molding cavity at a high temperature by a heated metal of low fusibility and high conductivity, exterior to the cavity and introducing the material into the cavity.

25. The process of casting materials in a mold which consists in maintaining the walls of the molding cavity at a high temperature by a heated metal of low fusibility and high boiling point, exterior to the cavity and introducing the material into the cavity.

26. The process of casting materials in a mold which consists in maintaining the walls of the molding cavity at a high temperature by a heated metal of low fusibility and high vaporizing point, exterior to the cavity and introducing the material into the cavity.

27. The process of casting ferrous metals in molds which consists in impregnating the molds with a metal gasifiable at a tem-

perature below the melting point of the metal cast, maintaining the walls of the molding cavity in contact with a material containing an additional amount of the gasifiable metal, and inserting the molten ferrous metal into the mold.

28. The process of casting ferrous metals which consists in impregnating the walls of the cavity with zinc while maintaining the heated walls in contact with a metal containing zinc, and inserting the molten ferrous metal into the mold.

29. The process of casting ferrous metals in molds which consists in impregnating the walls of the cavity of the mold with zinc, surrounding the walls with heated lead, and inserting the molten ferrous metal into the molds.

30. The process of casting ferrous metals which consists in impregnating the walls of the cavity with zinc, surrounding the walls with a metal containing zinc, and inserting the molten ferrous metal into the molds.

31. The process of casting ferrous metals in molds which consists in forcing a metal gasifiable at a temperature below the melting point of the metal cast through the wall of the mold by subjecting the said gasifiable metal to heat and pressure, and inserting the ferrous metal into the cavity of the mold.

32. The process of casting ferrous metals in molds which consists in forcing a metal gasifiable at a temperature below the melting point of the metal cast through the wall of the mold by subjecting the said gasifiable metal to heat and its vapor pressure, and inserting the ferrous metal into the cavity of the mold.

In testimony whereof, I have hereunto signed my name to this specification.

HUBERT A. MYERS.